

# UNITED STATES PATENT OFFICE.

EDWARD J. SCHRODER, OF CHICAGO, ILLINOIS.

## ROOFING.

1,188,495.

Specification of Letters Patent. Patented June 27, 1916.

No Drawing.

Application filed January 21, 1914. Serial No. 813,395.

To all whom it may concern:

Be it known that I, EDWARD J. SCHRODER, a citizen of the United States, residing at Chicago, in the county of Cook and State 5 of Illinois, have invented certain new and useful Improvements in Roofing, of which the following is a specification.

The article of commerce termed prepared or ready roofing comprises a sheet of suitable material saturated with asphalt or a similar waterproofing substance. A sheet material commonly used in roofing is that known as wool felt. In endeavoring to provide a cheap and satisfactory substitute for 10 wool felt, I have produced a felt of novel characteristics which is not only less expensive than wool felt, but possesses features of superiority thereto. The new felt contains chemical fiber from southern yellow pine, (long-leaf, loblolly and jack pine) 15 which are rich in resinous substances. The felt may consist entirely of such chemical resinous-wood fiber, or may contain a greater or less quantity of other fibers or 20 rags. I prefer that the felt should consist entirely of the wood fiber specified, but if it be desired to reduce the cost of the felt, other fibers or rags may be used in combination with the chemical southern yellow 25 pine fiber. The felt should, however, contain not less than fifty per cent. of chemical southern yellow pine fiber.

The new felt referred to is much stronger than wool felt. Prior to saturation, the 30 bursting strain, per square inch on a Mullen tester, of a sheet of average wool felt, is six-tenths pounds per one-thousandth of an inch in thickness, whereas the bursting strain of a sheet of the pure wood felt hereinbefore described is two and two-tenths 35 pounds per one-thousandth of an inch in thickness. The bursting strain of wood felt which does not consist wholly of chemical southern yellow pine fiber will vary according to the kinds of fibers and the relative proportions of the different sorts of fibers contained in the sheet.

The wood felt may be made in various 40 gages according to the character of the roofing to be made, the range in gage being from about 0.035 to 0.100. The gage and the weight of the wood felt are ordina-

rily so proportioned as to permit of the standard 150% saturation. The greater strength of wood felt as compared with 55 wool felt is of advantage in the manufacture of roofing, in that more tension can be put on the web for the purpose of making the web run straight, thus avoiding the damage and loss resulting when the web does 60 not run true. The additional strength is also beneficial in the practical use of the roofing.

My improved roofing material is able to absorb and retain as great an amount of 65 waterproofing material as wool felt. I attribute this characteristic to the fact that the fibers of southern resinous woods contain relatively large resin ducts which, being substantially emptied of resin in the 70 chemical process of producing wood pulp, are able to absorb and retain a correspondingly large amount of waterproofing.

The wood felt herein described is stiffer 75 than wool felt, its rigidity being especially advantageous in roofing intended to be laid in the form of shingles. Being relatively stiff, shingles having a body of wood felt such as that herein set forth are not so apt to be injured by the wind as are shingles formed of wool felt.

It will be seen that I have produced a substitute for wool felt which is not only cheaper but is superior to wool felt in strength, rigidity and wearing qualities.

I claim as my invention:

1. An improved roofing material comprising a wood felt containing not less than about fifty per cent. of chemical southern resinous-wood fiber, and impregnated with 90 a waterproofing substance.

2. An improved roofing material comprising a wood felt containing more than fifty per cent. of yellow pine fibers and impregnated with a waterproofing substance.

3. A roofing material consisting of a felted sheet of yellow pine fibers substantially saturated with constituents of coal tar.

In testimony whereof I affix my signature in the presence of two witnesses.

EDWARD J. SCHRODER.

Witnesses:

CHARLES W. HILLS, Jr.,  
GEORGE L. CHINDAHL.